# EUROPEAN PATENT SPECIFICATION

(11) **EP 0 952 485 B1**
(45) Date of publication and mention of the grant of the patent: **08.10.2003**
(21) Application number: 99201571.9
(22) Date of filing: 18.01.1999
(51) Int. Cl.: G03C 7/392, G03C 1/825

(54) **Color photographic element containing elemental silver and nitrogen heterocycle in a non-light sensitive layer**
Farbphotographisches Element mit elementarem Silber und stickstoffhaltigem Heterozyclus in einer lichtunempfindlichen Schicht
Elément photographique couleur contenant de l'argent élémentaire et hétérocycle azoté dans une couche non-sensible à la lumière

(30) Priority: 29.01.1998 US 14855; 05.11.1998 US 186844
(43) Date of publication of application: 27.10.1999
(62) Divisional of application: 99200145.3
(73) Proprietor: EASTMAN KODAK COMPANY, Rochester, New York 14650 (US)
(72) Inventor: Clark, Bernard A., c/o Eastman Kodak Company, Rochester, New York 14650-2201 (US); Boff, Jane Sarah, c/o Eastman Kodak Company, Rochester, New York 14650-2201 (US); Allway, Phillip Arthur c/o Eastman Kodak Company, Rochester, New York 14650-2201 (US); Friedrich, Louis Elbert, c/o Eastman Kodak Company, Rochester, New York 14650-2201 (US); Singer, Stephen Paul, c/o Eastman Kodak Company, Rochester, New York 14650-2201 (US)
(74) Representative: Haile, Helen Cynthia

(56) References cited:
- JP-A- 52 093 770
- JP-A- 52 093 771
- US-A- 5 246 823
- US-A- 5 508 154

## Description

### FIELD OF THE INVENTION

This invention relates to a color photographic element containing elemental silver and a certain nitrogen heterocycle compound in a non-light sensitive layer.

### BACKGROUND OF THE INVENTION

It has long been an object of silver halide-based color photographic materials to create an image of an object in an accurate manner, both in terms of color and image structure characteristics such as graininess and sharpness. It is well known that the perceived sharpness of photographic images can be degraded through halation effects; that is, the reflection and subsequent diffusion of light within the light capturing element; in particular, reflection from the support. It is well known to use antihalation layers between the support and the sensitized layers in films to reduce light reflection. To be effective, an antihalation layer contains materials that absorb light and prevent reflection. In general, it is highly desirable for the light absorbing materials to be totally removed from the film element (or otherwise made colorless) after development in order to avoid increased background density. One well known type of light absorbing material suitable for use in antihalation layers is colloidal or finely divided elemental or metallic silver (also referred to as 'grey' silver). This type of silver metal is in a filamentary form and, in such form, absorbs light across the visible spectrum appearing grey or black. It is generally easily removed from the film element by the normal bleaching and fixing steps used to remove imaging silver from the element. This silver metal is not light sensitive and does not contribute to image formation. For references, see T.H. James, The Theory of the Photographic Process, 4^{th} Edition, p. 579, US 3,434,839, JP 09-067122A2 and Y.J. Zahng et al, Chin. Chem. Lett. 7(7), 687-690(1996).

Another use of colloidal or finely divided elemental or metallic silver is as a blue light absorbing filter. This form, commonly referred to as Carey-Lea silver, differs from 'grey' silver by being spherical in form. For references, see F. Evva, J. Signalaufzeichnungmaterialien, 4(1), 43-60(1976) and G. Frens, Kolloid-Z.Z. Polym, 233(1-2), 922-9(1969). This material is generally located in a non-imaging layer (commonly referred to as a yellow filter layer) farther away from the exposing source than or "underneath" the blue light sensitive emulsion layer. The function of this layer is to absorb any blue light not captured by the blue sensitized layers, thus avoiding undesired exposure by blue light of the underlying green and red sensitized emulsion layers, which retain some inherent sensitivity to blue light.

A problem associated with the use of elemental silver in both antihalation and yellow filter layers is an undesired increase in fog in nearby imaging layers. During development, silver ions are released and/or made soluble from the imaging layer. These silver ions can migrate to a non-light sensitive layer where the elemental silver is present. The silver can serve as nuclei for the reduction of the migrating silver ions to silver metal with concurrent oxidation of developer to oxidized developer. This process is called solution physical development (for references, see T.H. James, ibid., Chapter 13) and is non-imagewise. The oxidized developer can diffuse out of the antihalation layer and back into the nearby imaging layer where it can react with the couplers present and form dye in a non-imagewise fashion. This process is often highly process sensitive and can lead to variations in Dmin during photofinishing.

Another problem with the use of elemental silver in non-imaging layers is that these layers can absorb inhibitor fragments and other silver absorbing materials. This results in lower effective concentrations of the free species in the imaging layers. Restricted diffusion of such species through the layer containing the elemental silver can also occur.

It is known that the solution physical development involving elemental silver can be modified by the use of additives. For example, GB 2280276 A1, DE 1949418, East German Patent 2006 91/6 and Japanese Patent Application (Kokai) JP 3-138639A2 all describe various classes of materials that are useful for controlling the properties of elemental silver. In particular, JP 6-347940 describes among others, the use of benzrotriazoles and other nitrogen heterocycles. However, in all of these references, the materials are water soluble and, of all the examples shown, the maximum ClogP is 3.79. Such water soluble materials can undesirably diffuse to imaging layers where they can cause inhibition of development and loss of sensitivity to light.

Solution physical development can be promoted by materials that form soluble silver salts. In particular, materials that release low molecular weight water solubilized thiols, which are used as bleach accelerators, can increase the amount of solution physical development. Couplers that release such thiols are known are bleach accelerator releasing couplers; for examples, see EP 193389, US 4,861,701; US 4,959,299; US 4,912,024; US 5,300,406 and US 5,358.828. It is also possible to release the same bleach accelerators from materials other than couplers by imagewise means that do not involve direct coupling with oxidized developer; for example, see US 4,684,604 or by non-imagewise means, for examples, see US 4,923,784, US 4,865,956 and US 5,019,492. Thus, increases in Dmin in imaging layers near to non-imaging layers which contain collodial silver are particularly problematic when bleach accelerators are also present.

Substituted triazoles, including 1,2,3-triazoles, 1,2,4-triazoles (including tetraazaindenes) and benzotriazoles, are commonly known in the art as inhibitor fragments and as antifoggants; for example, as in US 3,671,255. As inhibitor fragments, they are attached to a coupling moiety through a nitrogen atom and do not interact with silver until coupling occurs and the nitrogen atom is freed. As antifoggants, these materials are added directly to silver emulsions before coating of the film or added directly to the developer solutions. JP-60-29390 describes the use of ballasted benzotriazoles for use as inhibitor fragments attached to couplers to form Development Inhibitor Releasing Couplers (DIRs). U.S. Patent Nos. 5,275,931; 4,920,043; and 4,720,451, and Japanese Patent Applications (Kokai) JP-63-193147, JP-60-217358, JP-59-159162, JP-57-125939, JP-4-204937, JP-1-137255 all describe the use of various triazole and benzotriazole derivatives for use as antifoggants. U.S. Patent No. 5,508,154 describes the use of bicyclic heterocycles that contain a minimum of 4 nitrogen atoms as antifoggants in systems that contain inhibitor releasing couplers. DE 1 95 07913 A1 describes the use of ballasted benzimidazoles to improve granularity particularly with certain pyrazolone image couplers. EP 0 369 486 B I describes the use of various heterocyclic thiols with fine silver chloride emulsions to remove inhibiting species. US 4,871,658 describes the use of tetrazoles with silver iodobromide emulsions to decrease fog. All of these materials are used for control of imaging silver halide emulsions in light sensitive layers and are not used in non-imaging layers.

A problem to be solved is to provide a photographic element containing a non-light sensitive layer containing elemental silver which has a reduced tendency to increase the Dmin of nearby light sensitive layers.

### SUMMARY OF THE INVENTION

The invention provides a color photographic element comprising a non-light sensitive layer containing elemental silver and a nitrogen heterocycle compound having a ClogP of at least 4.5, which compound comprises a ring system of one or more fused rings containing at least one -N-H bond, the ring system comprising a total of at least three nitrogen ring members and the associated bonds; provided that the compound does not contain an -SH group or >C=S group and does not react with an oxidized developer.

The invention provides a reduction in Dmin values of the imaging layers.

### DETAILED DESCRIPTION OF THE INVENTION

The photographic element of the present invention is generally as described in the Summary of the Invention. Typically, it relates to a light sensitive color photographic element with at least one red sensitive silver halide emulsion layer containing at least one non-diffusing cyan coupler, at least one green sensitive silver halide emulsion layer having at least one non-diffusing magenta coupler and at least one blue sensitive silver halide emulsion layer having at least one non-diffusing yellow coupler, and at least one non-light sensitive layer containing both a form of elemental silver metal and a nitrogen heterocycle in accordance with the invention.

Suitable nitrogen heterocycles for use in this invention comprise a ring system of one or more fused rings containing at least one -N-H bond, the ring system comprising a total of at least three nitrogen ring members and the associated bonds; the compound does not contain an -SH group or >C=S group and does not react with an oxidized developer. An example of such a compound is represented by Formula I:

In Formula I, Q, X and Y may be any combination of nitrogen and carbon atoms necessary to complete a heterocyclic ring system with Z representing an optional series of nitrogen and carbon atoms with i = 0 or 1 such that the heterocyclic ring system contains at least three nitrogen atoms in total. The bonds (shown as dotted lines) between the nitrogen and carbon atoms are single or double as necessary to complete the ring. Any carbon atom that is present in the ring may have a hydrogen atom or other substitutent such as an alkyl group, a phenyl group, an ether group, a thioether group, a nitrogen group such as amino, aminocarbonyl or aminosulfonyl, an oxygen, a sulfoxide group, a sulfone group, a halide such a chloro or bromo, a cyano group, a nitro group, a carbonyl group such as keto, carboxylic acid, carboxylate ester or carbamoyl or such other substituent group as described generally hereafter. These substitutents may be connected to others to form additional ring systems and benzo-, naptho- or hetero- rings may be annulated to the heterocyclic ring nucleus. Triazole rings and diazole rings fused to one or more further azole rings are conveniently employed. Some examples of the ring systems of Formula I of the invention are 1,2,3 triazoles, 1,2,4 triazoles, benzotriazoles, tetraazaindenes, pentaazaindenes, purines, tetrazoles and pyrazolotriazoles.

Free thiol groups (-SH) and thiocarbonyl groups (>C=S) are specifically excluded as substitutents. At high levels, ballasted heterocyles with thiol or thiocarbonyl groups can form insoluble silver salts that cannot be removed from the film by the bleaching or fixing steps of the process. Retained silver salts are colored and result in degradation of color reproduction of the film.

The materials of Formula I are not couplers and do not react with oxidized developer. Such reaction would adversely affect for example, image forming efficiency and color.

An important feature of the heterocycles of Formula I is their oil/water partition coefficient. The oil/water partition coefficient can be calculated using the software program Medchem 3.54 to predict this value as ClogP (Calculated log partition coefficient). Medchem version 3.54 is a software program produced by the Medicinal Chemistry Project, Pomona College, Pomona California. It is believed that, in order to obtain the desired reduction of Dmin and fog in nearby imaging layers, the water solubility cannot be so low that the material is unable to interact effectively with the silver surface. Thus, it is preferred that the overall ClogP of the heterocycles of Formula I are not greater than 10.5 and most preferred that the ClogP is not greater than 10. It is also believed, however, that the water solubility cannot be so high that the material can diffuse away from the layer containing the elemental silver into adjacent imaging layers thereby causing a loss in light sensitivity. Thus, it is necessary that the ClogP of the heterocycle of Formula I be at least 4.5 or most preferably at least 5.5.

In general, the molar ratio of the heterocycle of Formula I to silver should be at least 0.1 mmole to mole of silver and more preferably, at least 1.0 mmole but less than 100 mmole and, more preferably, less than 50 mmole.

The following are examples of heterocycles that are useful in this invention along with the corresponding ClogP values in parentheses:

The heterocycles used in the invention are conveniently employed with the compounds typically used as scavengers for oxidized developer. Such scavengers are described in Research Disclosure as described hereinafter and include, for example, phenolic and hydroquinone derivatives such as 2,4-di-t-octylhydroquinone.

The materials of the invention can be added to a solution containing silver before coating or be mixed with the silver just prior to or during coating. In either case, additional components like dyes, doctors, surfactants, hardeners and other materials that are typically present in such solutions may also be present at the same time. The materials of the invention are not water soluble and cannot be added directly to the solution. They may be added directly if dissolved in an organic water miscible solution such as methanol, acetone or the like or more preferably as a dispersion. A dispersion incorporates the material in a stable, finely divided state in a hydrophobic organic solvent that is stabilized by suitable surfactants and surface active agents usually in combination with a binder or matrix such as gelatin. The dispersion may contain one or more permanent coupler solvens that dissolve the material and maintain it in a liquid state. Some examples of suitable permanent coupler solvents are tricresylphosphate, N,N-diethyllauramide, N,N'-dibutyllauramide, p-dodecylphenol, dibutylpthalate, di-n-butyl sebacate, N-n-butylacetanilide, 9-octadecen-1-ol, trioctylamine and 2-ethyl-hexylphosphate. The dispersion may require an auxiliary coupler solvent to initially dissolve the component but is removed afterwards, usually either by evaporation or by washing with additional water. Some examples of suitable auxiliary coupler solvents are ethyl acetate, cyclohexanone and 2-(2-butoxy-ethoxy)ethyl acetate. The dispersion may also be stabilized by addition of polymeric materials to form stable latexes. Examples of suitable polymers for this use generally contain water solubilizing groups or have regions of high hydrophilicity. Some examples of suitable dispersing agents or surfactants are Alkanol XC or saponin. The materials of the invention may also be dispersed as an admixture with another component of the system such as a dye or a oxidized developer scavenger so that both are present in the same oil droplet.

Throughout this specification, unless otherwise specifically stated, when a substituent group contains a substitutable hydrogen, it is intended to encompass not only the substituent's unsubstituted form, but also its form further substituted with any group or groups as herein mentioned, so long as the group does not destroy properties necessary for photographic utility. Suitably, a substituent group may be halogen or may be bonded to the remainder of the molecule by an atom of carbon, silicon, oxygen, nitrogen, phosphorous, or sulfur. The substituent may be, for example, halogen, such as chlorine, bromine or fluorine; nitro; hydroxyl; cyano; carboxyl; or groups which may be further substituted, such as alkyl, including straight or branched chain or cyclic alkyl, such as methyl, trifluoromethyl, ethyl, *t*-butyl, 3-(2,4-di-t-pentylphenoxy) propyl, and tetradecyl; alkenyl, such as ethylene, 2-butene; alkoxy, such as methoxy, ethoxy, propoxy, butoxy, 2-methoxyethoxy, *sec*-butoxy, hexyloxy, 2-ethyl-hexyloxy, tetradecyloxy, 2-(2,4-di-*t*-pentylphenoxy)ethoxy, and 2-dodecyloxyethoxy; aryl such as phenyl, 4-t-butylphenyl, 2,4,6-trimethylphenyl, naphthyl; aryloxy, such as phenoxy, 2-methylphenoxy, alpha- or beta-naphthyloxy, and 4-tolyloxy; carbonamido, such as acetamido, benzamido, butyramido, tetradecanamido, alpha-(2,4-di-*t*-pentylphenoxy)acetamido, alpha-(2,4-di-*t*-pentylphenoxy)butyramido, alpha-(3-pentadecylphenoxy)-hexanamido, alpha-(4-hydroxy-3-*t*-butylphenoxy)-tetradecanamido, 2-oxo-pyrrolidin-1-yl, 2-oxo-5-tetradecylpyrrolin-1-yl, N-methyltetradecanamido, N-succinimido, N-phthalimido, 2,5-dioxo-1-oxazolidinyl, 3-dodecyl-2,5-dioxo-1-imidazolyl, and N-acetyl-N-dodecylamino, ethoxycarbonylamino, phenoxycarbonylamino, benzyloxycarbonylamino, hexadecyloxycarbonylamino, 2,4-di-t-butylphenoxycarbonylamino, phenylcarbonylamino, 2,5-(di-*t*-pentylphenyl)carbonylamino, *p*-dodecylphenylcarbonylamino, *p*-tolylcarbonylamino, N-methylureido, N,N-dimethylureido, N-methyl-N-dodecylureido, N-hexadecylureido, N,N-dioctadecylureido, N,N-dioctyl-N'-ethylureido, N-phenylureido, N,N-diphenylureido, N-phenyl-N-*p*-tolylureido, N-(*m*-hexadecylphenyl)ureido, N,N-(2,5-di-*t*-pentylphenyl)-N'-ethylureido and *t*-butylcarbonamido; sulfonamido, such as methylsulfonamido, benzenesulfonamido, *p*-tolylsulfonamido, *p*-dodecylbenzenesulfonamido, N-methyltetradecylsulfonamido, N,N-dipropylsulfamoylamino and hexadecylsulfonamido; sulfamoyl, such as N-methylsulfamoyl, N-ethylsulfamoyl, N,N-dipropylsulfamoyl, N-hexadecylsulfamoyl, N,N-dimethylsulfamoyl; N-[3-(dodecyloxy)propyl]sulfamoyl, N-[4-(2,4-di-*t*-pentylphenoxy)butyl]-sulfamoyl, N-methyl-N-tetradecylsulfamoyl and N-dodecylsulfamoyl; carbamoyl, such as N-methylcarbamoyl, N,N-dibutylcarbamoyl, N-octadecylcarbamoyl, N-[4-(2,4-di-*t*-pentylphenoxy)butyl]carbamoyl, N-methyl-N-tetradecylcarbamoyl and N,N-dioctylcarbamoyl; acyl, such as acetyl, (2,4-di-t-amylphenoxy)acetyl, phenoxycarbonyl, *p*-dodecyloxyphenoxycarbonyl, methoxycarbonyl, butoxycarbonyl, tetradecyloxycarbonyl, ethoxycarbonyl, benzyloxycarbonyl, 3-pentadecyloxycarbonyl and dodecyloxycarbonyl; sulfonyl, such as methoxysulfonyl, octyloxysulfonyl, tetradecyloxysulfonyl, 2-ethylhexyloxysulfonyl, phenoxysulfonyl, 2,4-di-*t*-pentylphenoxysulfonyl, methylsulfonyl, octylsulfonyl, 2-ethylhexylsulfonyl, dodecylsulfonyl, hexadecylsulfonyl, phenylsulfonyl, 4-nonylphenylsulfonyl and *p*-tolylsulfonyl; sulfonyloxy, such as dodecylsulfonyloxy and hexadecylsulfonyloxy; sulfinyl, such as methylsulfinyl, octylsulfinyl, 2-ethylhexylsulfinyl, dodecylsulfinyl, hexadecylsulfinyl, phenylsulfinyl, 4-nonylphenylsulfinyl and *p*-tolylsulfinyl; thio, such as ethylthio, octylthio, benzylthio, tetradecylthio, 2-(2,4-di-*t*-pentylphenoxy)ethylthio, phenylthio, 2-butoxy-5-t-octylphenylthio and *p*-tolylthio; acyloxy, such as acetyloxy, benzoyloxy, octadecanoyloxy, *p*-dodecylamidobenzoyloxy, N-phenylcarbamoyloxy, N-ethylcarbamoyloxy and cyclohexylcarbonyloxy; amino, such as phenylanilino, 2-chloroanilino, diethylamino and dodecylamino; imino, such as 1-(N-phenylimido) ethyl, N-succinimido or 3-benzylhydantoinyl; phosphate, such as dimethylphosphate and ethylbutylphosphate; phosphite, such as diethyl and dihexylphosphite; a heterocyclic group, a heterocyclic oxy group or a heterocyclic thio group, each of which may be substituted and which contain a 3 to 7 membered heterocyclic ring composed of carbon atoms and at least one hetero atom selected from the group consisting of oxygen, nitrogen and sulfur, such as 2-furyl, 2-thienyl, 2-benzimidazolyloxy or 2-benzothiazolyl; quaternary ammonium, such as triethylammonium; and silyloxy, such as trimethylsilyloxy.

If desired, the substituents may themselves be further substituted one or more times with the described substituent groups. The particular substituents used may be selected by those skilled in the art to attain the desired photographic properties for a specific application and can include, for example, hydrophobic groups, solubilizing groups, blocking groups, releasing or releasable groups, etc. Generally, the above groups and substituents thereof may include those having up to 48 carbon atoms, typically 1 to 36 carbon atoms and usually less than 24 carbon atoms, but greater numbers are possible depending on the particular substituents selected.

The materials of the invention can be used in any of the ways and in any of the combinations known in the art. It is essential that the heterocyclic compounds used in the invention are incorporated in a non-sensitized layer on a support to form part of a photographic element.

To control the migration of various components, it may be desirable to include a high molecular weight or polymeric backbone containing hydrophobic or "ballast" group in molecules. Representative ballast groups include substituted or unsubstituted alkyl or aryl groups containing 8 to 48 carbon atoms. Representative substituents on such groups include alkyl, aryl, alkoxy, aryloxy, alkylthio, hydroxy, halogen, alkoxycarbonyl, aryloxycarbonyl, carboxy, acyl, acyloxy, amino, anilino, carbonamido, carbamoyl, alkylsulfonyl, arylsulfonyl, sulfonamido, and sulfamoyl groups wherein the substituents typically contain 1 to 42 carbon atoms. Such substituents can also be further substituted.

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

A typical multicolor photographic element comprises a support bearing a cyan dye image-forming unit comprised of at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one blue-sensitive silver halide emulsion layer having associated therewith at least one yellow dye-forming coupler. The element can contain additional layers, such as filter layers, interlayers, overcoat layers and subbing layers.

If desired, the photographic element can be used in conjunction with an applied magnetic layer as described in *Research Disclosure,* November 1992, Item 34390 published by Kenneth Mason Publications, Ltd., Dudley Annex, 12a North Street, Emsworth, Hampshire P010 7DQ, ENGLAND, and as described in Hatsumi Kyoukai Koukai Gihou No. 94-6023, published March 15, 1994, available from the Japanese Patent Office. When it is desired to employ the inventive materials in a small format film, Research Disclosure, June 1994, Item 36230, provides suitable embodiments.

In the following discussion of suitable materials for use in the emulsions and elements of this invention, reference will be made to Research Disclosure, September 1996, Item 38957, available as described above, which is referred to herein by the term "Research Disclosure". The Sections hereafter referred to are Sections of the Research Disclosure.

Except as provided, the silver halide emulsion containing elements employed in this invention can be either negative-working or positive-working as indicated by the type of processing instructions (i.e. color negative, reversal, or direct positive processing) provided with the element. Suitable emulsions and their preparation as well as methods of chemical and spectral sensitization are described in Sections I through V. Various additives such as UV dyes, brighteners, antifoggants, stabilizers, light absorbing and scattering materials, and physical property modifying addenda such as hardeners, coating aids, plasticizers, lubricants and matting agents are described, for example, in Sections II and VI through VIII. Color materials are described in Sections X through XIII. Suitable methods for incorporating couplers and dyes, including dipersions in organic solvents, are described in Section X(E). Scan facilitating is described in Section XIV. Supports, exposure, development systems, and processing methods and agents are described in Sections XV to XX. The information contained in the September 1994 Research Disclosure, Item No. 36544 referenced above, is updated in the September 1996 Research Disclosure, Item No. 38957. Certain desirable photographic elements and processing steps, including those useful in conjunction with color reflective prints, are described in Research Disclosure, Item 37038, February 1995.

Coupling-off groups are well known in the art. Such groups can determine the chemical equivalency of a coupler, i.e., whether it is a 2-equivalent or a 4-equivalent coupler, or modify the reactivity of the coupler. Such groups can advantageously affect the layer in which the coupler is coated, or other layers in the photographic recording material, by performing, after release from the coupler, functions such as dye formation, dye hue adjustment, development acceleration or inhibition, bleach acceleration or inhibition, electron transfer facilitation or color correction.

The presence of hydrogen at the coupling site provides a 4-equivalent coupler, and the presence of another coupling-off group usually provides a 2-equivalent coupler. Representative classes of such coupling-off groups include, for example, chloro, alkoxy, aryloxy, hetero-oxy, sulfonyloxy, acyloxy, acyl, heterocyclyl, sulfonamido, mercaptotetrazole, benzothiazole, mercaptopropionic acid, phosphonyloxy, arylthio and arylazo. These coupling-off groups are described in the art, for example, in U.S. Pat. Nos. 2,455,169, 3,227,551, 3,432,521, 3,476,563, 3,617,291, 3,880,661, 4,052,212 and 4,134,766; and in UK. Patents and published application Nos. 1,466,728, 1,531,927, 1,533,039, 2,006,755A and 2,017,704A.

Image dye-forming couplers may be included in the element such as couplers that form cyan dyes upon reaction with oxidized color developing agents which are described in such representative patents and publications as: "Farbkuppler-eine Literature Übersicht," published in Agfa Mitteilungen, Band III, pp. 156-175 (1961) as well as in U.S. Patent Nos. 2,367,531; 2,423,730; 2,474,293; 2,772,162; 2,895,826; 3,002,836; 3,034,892; 3,041,236; 4,333,999; 4,746,602; 4,753,871; 4,770,988; 4,775,616; 4,818,667; 4,818,672; 4,822,729; 4,839,267; 4,840,883; 4,849,328; 4,865,961; 4,873,183; 4,883,746; 4,900,656; 4,904,575; 4,916,051; 4,921,783; 4,923,791; 4,950,585; 4,971,898; 4,990,436; 4,996,139; 5,008,180; 5,015,565; 5,011,765; 5,011,766; 5,017,467; 5,045,442; 5,051,347; 5,061,613; 5,071,737; 5,075,207; 5,091,297; 5,094,938; 5,104,783; 5,178,993; 5,813,729; 5,187,057; 5,192,651; 5,200,305 5,202,224; 5,206,130; 5,208,141; 5,210,011; 5,215,871; 5,223,386; 5,227,287; 5,256,526; 5,258,270; 5,272,051; 5,306,610; 5,326,682; 5,366,856; 5,378,596; 5,380,638; 5,382,502; 5,384,236; 5,397,691; 5,415,990; 5,434,034; 5,441,863; EPO 0 246 616; EPO 0 250 201; EPO 0 271 323; EPO 0 295 632; EPO 0 307 927; EPO 0 333 185; EPO 0 378 898; EPO 0 389 817; EPO 0 487 111; EPO 0 488 248; EPO 0 539 034; EPO 0 545 300; EPO 0 556 700; EPO 0 556 777; EPO 0 556 858; EPO 0 569 979; EPO 0 608 133; EPO 0 636 936; EPO 0 651 286; EPO 0 690 344; German OLS 4,026,903; German OLS 3,624,777. and German OLS 3,823,049. Typically such couplers are phenols, naphthols, or pyrazoloazoles.

Couplers that form magenta dyes upon reaction with oxidized color developing agent are described in such representative patents and publications as: "Farbkuppler-eine Literature Übersicht," published in Agfa Mitteilungen, Band III, pp. 126-156 (1961) as well as U.S. Patents 2,311,082 and 2,369,489; 2,343,701; 2,600,788; 2,908,573; 3,062,653; 3,152,896; 3,519,429; 3,758,309; 3,935,015; 4,540,654; 4,745,052; 4,762,775; 4,791,052; 4,812,576; 4,835,094; 4,840,877; 4,845,022; 4,853,319; 4,868,099; 4,865,960; 4,871,652; 4,876,182; 4,892,805; 4,900,657; 4,910,124; 4,914,013; 4,921,968; 4,929,540; 4,933,465; 4,942,116; 4,942,117; 4,942,118; U.S. Patent 4,959,480; 4,968,594; 4,988,614; 4,992,361; 5,002,864; 5,021,325; 5,066,575; 5,068,171; 5,071,739; 5,100,772; 5,110,942; 5,116,990; 5,118,812; 5,134,059; 5,155,016; 5,183,728; 5,234,805; 5,235,058; 5,250,400; 5,254,446; 5,262,292; 5,300,407; 5,302,496; 5,336,593; 5,350,667; 5,395,968; 5,354,826; 5,358,829; 5,368,998; 5,378,587; 5,409,808; 5,411,841; 5,418,123; 5,424,179; EPO 0 257 854; EPO 0 284 240; EPO 0 341 204; EPO 347,235; EPO 365,252; EPO 0 422 595; EPO 0 428 899; EPO 0 428 902; EPO 0 459 331; EPO 0 467 327; EPO 0 476 949; EPO 0 487 081; EPO 0 489 333; EPO 0 512 304; EPO 0 515 128; EPO 0 534 703; EPO 0 554 778; EPO 0 558 145; EPO 0 571 959; EPO 0 583 832; EPO 0 583 834; EPO 0 584 793; EPO 0 602 748; EPO 0 602 749; EPO 0 605 918; EPO 0 622 672; EPO 0 622 673; EPO 0 629 912; EPO 0 646 841, EPO 0 656 561; EPO 0 660 177; EPO 0 686 872; WO 90/10253; WO 92/09010; WO 92/10788; WO 92/12464; WO 93/01523; WO 93/02392; WO 93/02393; WO 93/07534; UK Application 2,244,053; Japanese Application 03192-350; German OLS 3,624,103; German OLS 3,912,265; and German OLS 40 08 067. Typically such couplers are pyrazolones, pyrazoloazoles or pyrazolobenzimidazoles that form magenta dyes upon reaction with oxidized color developing agents.

Couplers that form yellow dyes upon reaction with oxidized color developing agent are described in such representative patents and publications as: "Farbkuppler-eine Literature Übersicht," published in Agfa Mitteilungen; Band III; pp. 112-126(1961); as well as U.S. Patent 2,298,443; 2,407,210; 2,875,057; 3,048,194; 3,265,506; 3,447,928; 4,022,620; 4,443,536; 4,758,501; 4,791,050; 4,824,771; 4,824,773; 4,855,222; 4,978,605; 4,992,360; 4,994,361; 5,021,333; 5,053,325; 5,066,574; 5,066,576; 5,100,773; 5,118,599; 5,143,823; 5,187,055; 5,190,848; 5,213,958; 5,215,877; 5,215,878; 5,217,857; 5,219,716; 5,238,803; 5,283,166; 5,294,531; 5,306,609; 5,328,818; 5,336,591; 5,338,654; 5,358,835; 5,358,838; 5,360,713; 5,362,617; 5,382,506; 5,389,504; 5,399,474;. 5,405,737; 5,411,848; 5,427,898; EPO 0 327 976; EPO 0 296 793; EPO 0 365 282; EPO 0 379 309; EPO 0 415 375; EPO 0 437 818; EPO 0 447 969; EPO 0 542 463; EPO 0 568 037; EPO 0 568 196; EPO 0 568 777; EPO 0 570 006; EPO 0 573 761; EPO 0 608 956; EPO 0 608 957; and EPO 0 628 865. Such couplers are typically open chain ketomethylene compounds.

Couplers that form colorless products upon reaction with oxidized color developing agent are described in such representative patents as: UK. 861,138; U.S. Pat. Nos. 3,632,345; 3,928,041; 3,958,993 and 3,961,959. Typically such couplers are cyclic carbonyl containing compounds that form colorless products on reaction with an oxidized color developing agent.

Couplers that form black dyes upon reaction with oxidized color developing agent are described in such representative patents as U.S. Patent Nos. 1,939,231; 2,181,944; 2,333,106 and 4,126,461; German OLS No. 2,644,194 and German OLS No. 2,650,764. Typically, such couplers are resorcinols or m-aminophenols that form black or neutral products on reaction with oxidized color developing agent.

In addition to the foregoing, so-called "universal" or "washout" couplers may be employed. These couplers do not contribute to image dye-formation. Thus, for example, a naphthol having an unsubstituted carbamoyl or one substituted with a low molecular weight substituent at the 2- or 3- position may be employed. Couplers of this type are described, for example, in U.S. Patent Nos. 5,026,628, 5,151,343 and 5,234,800.

It may be useful to use a combination of couplers any of which may contain known ballasts or coupling-off groups such as those described in U.S. Patent 4,301,235; U.S. Patent 4,853,319 and U.S. Patent 4,351,897. The coupler may contain solubilizing groups such as described in U.S. Patent 4,482,629. The coupler may also be used in association with "wrong" colored couplers (e.g. to adjust levels of interlayer correction) and, in color negative applications, with masking couplers such as those described in EP 213.490; Japanese Published Application 58-172,647; U.S. Patent Nos. 2,983,608; 4,070,191; and 4,273,861; German Applications DE 2,706,117 and DE 2,643,965; UK. Patent 1,530,272 and Japanese Application 58-113935. The masking couplers may be shifted or blocked, if desired.

The invention materials may be used in association with materials that release Photographically Useful Groups (PUGS) that accelerate or otherwise modify the processing steps e.g. of bleaching or fixing to improve the quality of the image. These bleach releasing materials may or may not be couplers as described in the background. Bleach accelerator releasing couplers such as those described in EP 193,389; EP 301,477; U.S. 4,163,669; U.S. 4,865,956; and U.S. 4,923,784, may be useful. Also contemplated is use of the compositions in association with nucleating agents, development accelerators or their precursors (UK Patent 2,097,140; UK. Patent 2,131,188); electron transfer agents (U.S. 4,859,578; U.S. 4,912,025); antifogging and anti color-mixing agents such as derivatives of hydroquinones, aminophenols, amines, gallic acid; catechol; ascorbic acid; hydrazides; sulfonamidophenols and non color-forming couplers.

The invention materials may also be used in combination with filter dye layers comprising colloidal silver sol or yellow, cyan, and/or magenta filter dyes, either as oil-in-water dispersions, latex dispersions or as solid particle dispersions. Additionally, they may be used with "smearing" couplers (e.g. as described in U.S. 4,366,237; EP 96,570; U.S. 4,420,556; and U.S. 4,543,323.) Also, the compositions may be blocked or coated in protected form as described, for example, in Japanese Application 61/258,249 or U.S. 5,019,492.

The invention materials may further be used in combination with image-modifying compounds that release PUGS such as "Developer Inhibitor-Releasing" compounds (DIRs). DIRs useful in conjunction with the compositions of the invention are known in the art and examples are described in U.S. Patent Nos. 3,137,578; 3,148,022; 3,148,062; 3,227,554; 3,384,657; 3,379,529; 3,615,506; 3,617,291; 3,620,746; 3,701,783; 3,733,201; 4,049,455; 4,095,984; 4,126,459; 4,149,886; 4,150,228; 4,211,562; 4,248,962; 4,259,437; 4,362,878; 4,409,323; 4,477,563; 4,782,012; 4,962,018; 4,500,634; 4,579,816; 4,607,004; 4,618,571; 4,678,739; 4,746,600; 4,746,601; 4,791,049; 4,857,447; 4,865,959; 4,880,342; 4,886,736; 4,937,179; 4,946,767; 4,948,716; 4,952,485; 4,956,269; 4,959,299; 4,966,835; 4,985,336 as well as in patent publications GB 1,560,240; GB 2,007,662; GB 2,032,914; GB 2,099,167; DE 2,842,063, DE 2,937,127; DE 3,636,824; DE 3,644,416 as well as the following European Patent Publications: 272,573; 335,319; 336,411; 346, 899; 362, 870; 365,252; 365,346; 373,382; 376,212; 377,463; 378,236; 384,670; 396,486; 401,612; 401,613.

Such compounds are also disclosed in "Developer-Inhibitor-Releasing (DIR) Couplers for Color Photography," C.R. Barr, J.R. Thirtle and P.W. Vittum in *Photographic Science and Engineering,* Vol. 13, p. 174 (1969). Generally, the developer inhibitor-releasing (DIR) couplers include a coupler moiety and an inhibitor coupling-off moiety (IN). The inhibitor-releasing couplers may be of the time-delayed type (DIAR couplers) which also include a timing moiety or chemical switch which produces a delayed release of inhibitor. Examples of typical inhibitor moieties are: oxazoles, thiazoles, diazoles, triazoles, oxadiazoles, thiadiazoles, oxathiazoles, thiatriazoles, benzotriazoles, tetrazoles, benzimidazoles, indazoles, isoindazoles, mercaptotetrazoles, selenotetrazoles, mercaptobenzothiazoles, selenobenzothiazoles, mercaptobenzoxazoles, selenobenzoxazoles, mercaptobenzimidazoles, selenobenzimidazoles, benzodiazoles, mercaptooxazoles, mercaptothiadiazoles, mercaptothiazoles, mercaptotriazoles, mercaptooxadiazoles, mercaptodiazoles, mercaptooxathiazoles, telleurotetrazoles or benzisodiazoles. In a preferred embodiment, the inhibitor moiety or group is selected from the following formulae: wherein R_{I} is selected from the group consisting of straight and branched alkyls of from 1 to about 8 carbon atoms, benzyl, phenyl, and alkoxy groups and such groups containing none, one or more than one such substituent; R_{II} is selected from R_{I} and -SR_{I}; R_{III} is a straight or branched alkyl group of from 1 to about 5 carbon atoms and m is from 1 to 3; and R_{IV} is selected from the group consisting of hydrogen, halogens and alkoxy, phenyl and carbonamido groups, -COOR_{V} and -NHCOOR_{V}, wherein R_{V} is selected from substituted and unsubstituted alkyl and aryl groups.

Although it is typical that the coupler moiety included in the developer inhibitor-releasing coupler forms an image dye corresponding to the layer in which it is located, it may also form a different color as one associated with a different film layer. It may also be useful that the coupler moiety included in the developer inhibitor-releasing coupler forms colorless products and/or products that wash out of the photographic material during processing (so-called "universal" couplers).

A compound such as a coupler may release a PUG directly upon reaction of the compound during processing, or indirectly through a timing or linking group. A timing group produces the time-delayed release of the PUG such groups using an intramolecular nucleophilic substitution reaction (U.S. 4,248,962); groups utilizing an electron transfer reaction along a conjugated system (U.S. 4,409,323; 4,421,845; 4,861,701, Japanese Applications 57-188035; 58-98728; 58-209736; 58-209738); groups that function as a coupler or reducing agent after the coupler reaction (U.S. 4,438,193; U.S. 4,618,571) and groups that combine the features describe above. It is typical that the timing group is of one of the formulae: wherein IN is the inhibitor moiety, Z is selected from the group consisting of nitro, cyano, alkylsulfonyl; sulfamoyl (-SO₂NR₂); and sulfonamido (-NRSO₂R) groups; n is 0 or 1; and R_{VI} is selected from the group consisting of substituted and unsubstituted alkyl and phenyl groups. The oxygen atom of each timing group is bonded to the coupling-off position of the respective coupler moiety of the DIAR.

The timing or linking groups may also function by electron transfer down an unconjugated chain. Linking groups are known in the art under various names. Often they have been referred to as groups capable of utilizing a hemiacetal or iminoketal cleavage reaction or as groups capable of utilizing a cleavage reaction due to ester hydrolysis such as U.S. 4,546,073. This electron transfer down an unconjugated chain typically results in a relatively fast decomposition and the production of carbon dioxide, formaldehyde or other low molecular weight by-products. The groups are exemplified in EP 464,612, EP 523,451, U.S. 4,146,396, Japanese Kokai 60-249148 and 60-249149.

Aside from the compound of Formula II of the invention, suitable developer inhibitor-releasing couplers that may be included in photographic light sensitive emulsion layer include, but are not limited to, the following:

Especially useful in this invention are tabular grain silver halide emulsions. Tabular grains are those having two parallel major crystal faces and having an aspect ratio of at least 2. The term "aspect ratio" is the ratio of the equivalent circular diameter (ECD) of a grain major face divided by its thickness (t). Specifically contemplated tabular grain emulsions are those in which greater than 50 percent of the total projected area of the emulsion grains are accounted for by tabular grains having a thickness of less than 0.3 micrometer (0.5 micrometer for blue sensitive emulsion) and an average tabularity (T) of greater than 25 (preferably greater than 100), where the term "tabularity" is employed in its art recognized usage as

T = ECD/t²

where
ECD is the average equivalent circular diameter of the tabular grains in micrometers and
t is the average thickness in micrometers of the tabular grains.

The average useful ECD of photographic emulsions can range up to about 10 micrometers, although in practice emulsion ECDs seldom exceed about 4 micrometers. Since both photographic speed and granularity increase with increasing ECDs, it is generally preferred to employ the smallest tabular grain ECDs compatible with achieving aim speed requirements.

Emulsion tabularity increases markedly with reductions in tabular grain thickness. It is generally preferred that aim tabular grain projected areas be satisfied by thin (t < 0.2 micrometer) tabular grains. To achieve the lowest levels of granularity it is preferred that aim tabular grain projected areas be satisfied with ultrathin (t <0.07 micrometer) tabular grains. Tabular grain thicknesses typically range down to about 0.02 micrometer. However, still lower tabular grain thicknesses are contemplated. For example, Daubendiek et al U.S. Patent 4,672,027 reports a 3 mole percent iodide tabular grain silver bromoiodide emulsion having a grain thickness of 0.017 micrometer. Ultrathin tabular grain high chloride emulsions are disclosed by Maskasky U.S. 5,217,858.

As noted above tabular grains of less than the specified thickness account for at least 50 percent of the total grain projected area of the emulsion. To maximize the advantages of high tabularity it is generally preferred that tabular grains satisfying the stated thickness criterion account for the highest conveniently attainable percentage of the total grain projected area of the emulsion. For example, in preferred emulsions, tabular grains satisfying the stated thickness criteria above account for at least 70 percent of the total grain projected area. In the highest performance tabular grain emulsions, tabular grains satisfying the thickness criteria above account for at least 90 percent of total grain projected area.

Suitable tabular grain emulsions can be selected from among a variety of conventional teachings, such as those of the following: Research Disclosure, Item 22534, January 1983, published by Kenneth Mason Publications, Ltd., Emsworth, Hampshire P010 7DD, England; U.S. Patent Nos. 4,439,520; 4,414,310; 4,433,048; 4,643,966; 4,647,528; 4,665,012; 4,672,027; 4,678,745; 4,693,964; 4,713,320; 4,722,886; 4,755,456; 4,775,617; 4,797,354; 4,801,522; 4,806,461; 4,835,095; 4,853,322; 4,914,014; 4,962,015; 4,985,350; 5,061,069 and 5,061,616. Tabular grain emulsions consisting predominantly of silver chloride are useful and are described, for example, in U.S. 5,310,635; 5,320,938; and 5,356,764.

The major faces of the tabular grains can lie in either {111} or {100} crystal planes. The mean ECD of tabular grain emulsions rarely exceeds 10 micrometers and more typically is less than 5 micrometers. In their most widely used form tabular grain emulsions are high bromide {111} } tabular grain emulsions. Such emulsions are illustrated by Kofron et al U.S. Patent 4,439,520, Wilgus et al U.S. Patent 4,434,226, Solberg et al U.S. Patent 4,433,048, Maskasky U.S. Patents 4,435,501, 4,463,087 and 4,173,320, Daubendiek et al U.S. Patents 4,414,310 and 4,914,014, Sowinski et al U.S. Patent 4,656,122, Piggin et al U.S. Patents 5,061,616 and 5,061,609, Tsaur et al U.S. Patents 5,147,771, '772, '773, 5,171,659 and 5,252,453, Black et al 5,219,720 and 5,334,495, Delton U.S. Patents 5,310,644, 5,372,927 and 5,460,934, Wen U.S. Patent 5,470,698, Fenton et al U.S. Patent 5,476,760, Eshelman et al U.S. Patents 5,612,,175 and 5,614,359, and Irving et al U.S. Patent 5,667,954.

Ultrathin high bromide {111} tabular grain emulsions are illustrated by Daubendiek et al U.S. Patents 4,672,027, 4,693,964, 5,494,789, 5,503,971 and 5,576,168, Antoniades et al U.S. Patent 5,250,403, Olm et al U.S. Patent 5,503,970, Deaton et al U.S. Patent 5,582,965, and Maskasky U.S. Patent 5,667,955.

High bromide {100} tabular grain emulsions are illustrated by Mignot U.S. Patents 4,386,156 and 5,386,156.

High chloride {111} tabular grain emulsions are illustrated by Wey U.S. Patent 4,399,215, Wey et al U.S. Patent 4,414,306, Maskasky U.S. Patents 4,400,463, 4,713,323, 5,061,617, 5,178,997, 5,183,732, 5,185,239, 5,399,478 and 5,411,852, and Maskasky et al U.S. Patents 5,176,992 and 5,178,998. Ultrathin high chloride {111} tabular grain emulsions are illustrated by Maskasky U.S. Patents 5,271,858 and 5,389,509.

High chloride {100} tabular grain emulsions are illustrated by Maskasky U.S. Patents 5,264,337, 5,292,632, 5,275,930 and 5,399,477, House et al U.S. Patent 5,320,938, Brust et al U.S. Patent 5,314,798, Szajewski et al U.S. Patent 5,356,764, Chang et al U.S. Patents 5,413,904 and 5,663,041, Oyamada U.S. Patent 5,593,821, Yamashita et al U.S. Patents 5,641,620 and 5,652,088, Saitou et al U.S. Patent 5,652,089, and Oyamada et al U.S. Patent 5,665,530. Ultrathin high chloride {100} tabular grain emulsions can be prepared by nucleation in the presence of iodide, following the teaching of House et al and Chang et al, cited above.

The emulsions can be surface-sensitive emulsions, i.e., emulsions that form latent images primarily on the surfaces of the silver halide grains, or the emulsions can form internal latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent. Tabular grain emulsions of the latter type are illustrated by Evans et al. U.S. 4,504,570.

Photographic elements can be exposed to actinic radiation, typically in the visible region of the spectrum, to form a latent image and can then be processed to form a visible dye image. Processing to form a visible dye image includes the step of contacting the element with a color developing agent to reduce developable silver halide and oxidize the color developing agent. Oxidized color developing agent in turn reacts with the coupler to yield a dye.

With negative-working silver halide, the processing step described above provides a negative image. One type of such element, referred to as a color negative film, is designed for image capture. Speed (the sensitivity of the element to low light conditions) is usually critical to obtaining sufficient image in such elements. Such elements are typically silver bromoiodide emulsions and may be processed, for example, in known color negative processes such as the Kodak C-41 process as described in The British Journal of Photography Annual of 1988, pages 191-198. If a color negative film element is to be subsequently employed to generate a viewable projection print as for a motion picture, a process such as the Kodak ECN-2 process described in the H-24 Manual available from Eastman Kodak Co. may be employed to provide the color negative image on a transparent support. Color negative development times are typically 3' 15" or less and desirably 90 or even 60 seconds or less.

The photographic element of the invention can be incorporated into exposure structures intended for repeated use or exposure structures intended for limited use, variously referred to by names such as "single use cameras", "lens with film" or "photosensitive material package units".

A reversal element is capable of forming a positive image without optical printing. To provide a positive (or reversal) image, the color development step is preceded by development with a non-chromogenic developing agent to develop exposed silver halide, but not form dye, and followed by uniformly fogging the element to render unexposed silver halide developable. Such reversal emulsions are typically sold with instructions to process using a color reversal process such as the Kodak E-6 process. Alternatively, a direct positive emulsion can be employed to obtain a positive image.

The above emulsions are typically sold with instructions to process using the appropriate method such as the mentioned color negative (Kodak C-41) or reversal (Kodak E-6) process.

Preferred color developing agents are *p*-phenylenediamines such as:
4-amino-N,N-diethylaniline hydrochloride,
4-amino-3-methyl-N,N-diethylaniline hydrochloride,
4-amino-3-methyl-N-ethyl-N-(2-methanesulfonamidoethyl)aniline sesquisulfate hydrate,
4-amino-3-methyl-N-ethyl-N-(2-hydroxyethyl)aniline sulfate,
4-amino-3-(2-methanesulfonamidoethyl)-N,N-diethylaniline hydrochloride, and
4-amino-N-ethyl-N-(2-methoxyethyl)-*m*-toluidine di-*p*-toluene sulfonic acid.

Development is usually followed by the conventional steps of bleaching, fixing, or bleach-fixing, to remove silver or silver halide, washing, and drying.

### Synthesis

The synthesis of H-A is shown in the following Scheme I as follows:

Synthesis of H-A: A stirred solution of Compound 1 (11.2g, 50mmol) in tetrahydrofuran (75ml) was cooled to -7°C. A mixture of Compound 2 (15.0g, 49mmol) in tetrahydrofuran (50ml) and pyridine (25ml) was added to the stirred solution over 0.5 hour keeping the temperature at -1°C. The reaction mixture was stirred at room temperature for 17 hours. The mixture was concentrated under reduced pressure and the residual oil was poured into a mixture of ice/water (500ml) and concentrated hydrochloric acid (100ml). The aqueous mixture was extracted with ethyl acetate (200ml) and the extract dried over magnesium sulphate and concentrated under reduced pressure to give a gum. A solution of potassium hydroxide (2.8g, 50mmol) in methanol (20ml) was added to a stirred solution of the gum dissolved in methanol (150ml). After stirring at room temperature for 0.25 hour, the solution was poured into 3N hydrochloric acid (300ml). The aqueous solution was extracted with ethyl acetate (2 x 150ml) and the extract dried over magnesium sulphate and concentrated under reduced pressure. The crude material was purified by column chromatography eluting with 1:9 60-80 petroleum ether : ethyl acetate to give a glass. The glass was crystallized from ethyl acetate (100ml) / 60-80 petroleum ether (20ml) to give a pale pink solid, 14.2g (63%). Expected C, 71.96; H, 8.50; N, 12.44; Found C, 71.54; H, 8.35; N, 12.37%.

### Photographic Examples

### A- Antihalation Layer

Bilayer photographic elements were prepared by coating the following layers on a cellulose triacetate film support (coverages are in g/m²). Unless otherwise noted, all comparative and inventive compounds were dispersed in twice their own weight of N,N-dibutyllauramide:
- Layer 1: (Antihalation Layer): Gelatin at 2.04, black colloidal silver at 0.135, UV-1 at 0.075 and UV-2 at 0.075. The inventive and comparative materials, when present, were added at 0.0081. ILS-1, when present, was added at 0.162.
- Layer 2: (Cyan Layer): gelatin at 1.61, C-1 at 0.48, C-2 at 0.075, C-3 at 0.015 and 0.683 red sensitized AgIBr tabular emulsion.
- Layer 3: (Overcoat): gelatin at 5.38 and 0.016 bis-vinylsulfonemethylether

The structures of the couplers and comparative materials used, along with the corresponding ClogP where appropriate, in the above format are as follows:

Samples of each element were given a stepped exposure and processed in the KODAK FLEXICOLOR (C41) process as described in British Journal of Photography Annual, 1988, pp196-198. Contrast of the elements was determined using the maximum slope between any two density points. Relative red sensitivity, a measure of speed, was determined by measuring the speed point +0.15 density units above Dmin and normalizing to the check position. Results are shown in Table I.

**TABLE I**

| **Use of Nitrogen Heterocycles a Antihalation Layers - Bilayer Format** | | | | | | |
|---|---|---|---|---|---|---|
| Sample | Comp/Inv | Additive | Red Dmin | Contrast | Relative Red Sensitivity | ClogP |
| BL-1 | Comp | None | 0.210 | 1.11 | 1.00 | |
| BL-2 | Comp | ILS-1 | 0.150 | 1.11 | 1.02 | |
| BL-3 | Comp | CH-1 | 0.124 | 1.08 | 0.90 | 4.22 |
| | | | | | | |
| BL-4 | Inv | H-A | 0.129 | 1.07 | 1.01 | 7.78 |
| BL-5 | Inv | H-A + ILS-1 | 0.105 | 1.08 | 1.02 | 7.78 |
| BL-6 | Inv | H-T | 0.183 | 1.12 | 1.01 | 11.25 |
| BL-7 | INV | H-U | 0.116 | 0.96 | 0.99 | 4.80 |
| BL-8 | Inv | H-U+ ILS-1 | 0.092 | 0.91 | 0.99 | 4.80 |

Sample BL-2 shows the effect of adding a hydroquinone scavenger for oxidized developer to the antihalation layer, a common method for removing unwanted oxidized developer. However, this alternative is not as effective at lowering red Dmin as are the compounds of the invention. BL-3 demonstrates that the ClogP must be sufficiently high to prevent wandering of the heterocycle into imaging layers and causing losses in light sensitivity. This sample achieves reducion in Dmin but exhibits an undesired reduction in Relative Red Sensitivity at the same time. Samples BL-4 to BL-8 show that the compounds of the invention are useful for controlling the Dmin of adjacent layers without significantly affecting their light sensitivity. Samples BL-5 and BL-8 show that the combination of the inventive materials with an oxidized developer scavenger is even more effective.

### B- Yellow Filter Layer:

In order to show the effect of the inventive materials in yellow filter layers containing Carey-Lea colloidal silver, four-layer photographic elements were prepared by coating the following layers on a cellulose triacetate film support containing a sublayer of 2.41 gelatin and 0.344 grey colloidal silver (all coverages are in g/m²). The coatings were exposed to blue and green light and processed as previously described. Results are shown in Table II.
- Layer 1: (Magenta Layer): 2.69 Gelatin, 0.0448 M-1, 0.0027 M-2 and 0.699 green sensitized AgIBr tabular emulsion.
- Layer 2: (Yellow Filter Layer): 0.645 Gelatin and ILS-1 (when present) at 0.086, ILS-2 (when present) at 0.054, H-A (when present) at 0.005, YFD-1 (when present) at 0.108 or Carey-Lea silver (when present) at 0.059.
- Layer 3: (Yellow Layer): 2.69 Gelatin, 0.968 Y-1, 0.054 Y-2 and 0.699 blue sensitized AgIBr tabular emulsion.
- Layer 4: (Overcoat): 2.69 Gelatin and 0.018 bis-vinylsulfonemethylether.

The structures of the couplers and comparative materials used, along with the corresponding ClogP where appropriate, in the above format are as follows:

**TABLE II**

| **Use of Nitrogen Heterocycles in Yellow Filter Layers - Four Layer Format** | | | | | |
|---|---|---|---|---|---|
| Sample | Comp/Inv | Yellow Filter Material | Additive | Blue Dmin | Green Dmin |
| FL-1 | Comp | YFD-1 | ILS-1 | 0.200 | 0.356 |
| FL-2 | Comp | YFD-1 | ILS-1 + H-A | 0.200 | 0.356 |
| FL-3 | Comp | YFD-1 | ILS-2 | 0.203 | 0.353 |
| FL-4 | Comp | YFD-1 | ILS-2 + H-A | 0.203 | 0.358 |
| FL-5 | Comp | Cary-Lea Ag | ILS-1 | 0.229 | 0.409 |
| FL-6 | Comp | Carey-Lea Ag | ILS-2 | 0.249 | 0.403 |
| | | | | | |
| FL-7 | Inv | Carey-Lea Ag | ILS-1 + H-A | 0.224 | 0.390 |
| FL-8 | Inv | Carey-Lea Ag | ILS-2 + H-A | 0.239 | 0.387 |

Comparison of samples FL-5 and FL-6 with FL-1 and FL-3 show that the presence of Carey-Lea colloidal elemental silver in place of organic yellow filter dye YFD-1 results in an increase in the Dmin of adjacent imaging layers. Addition of H-A to filter dye containing layers (FL-2 and FL-4) does not affect Dmin in adjacent layers. Only when the inventive heterocycle and elemental silver are present in the same layer are the adjacent Dmins reduced.

### C-Multilayer Photographic Examples

The invention can be further illustrated in the following multilayer experiments. Component laydowns are provided in units of gm/m².
**Layer A** (Protective Overcoat Layer).
**Layer B** (UV Filter Layer)

### Blue Sensitized Layer

**Layer C** (Yellow filter layer): ILS-1 at 0.054 and gelatin at 0.807.

### Green Sensitized Layer

**Layer D** (Interlayer): ILS-1 at 0.075 and gelatin at 0538.

### Red Sensitized Layer

**Layer E** (Interlayer): gelatin at 0.538 and ILS-1 at 0.076.
**Layer F** (Antihalation layer): gelatin at 1.61 and UV-1 and UV-2 both at 0.076.

Bislvinylsulfonyl)methane hardener was added at 1.55% of total gelatin weight. Antifoggants (including 4-hydroxy-6-methyl- 1,3,3a,7-tetraazaindene), surfactants, coating aids, coupler solvents, emulsion addenda, sequestrants, lubricants, matte and tinting dyes were added to the appropriate layers as is common in the art. The structures of the additional compounds used in the multilayer examples are as follows.

Multilayer examples ML-1 to 8 which all employ the same basic formula with variations in the AHU with and without an interlayer are summarized in Table III. Samples of each element were given a stepped exposure and processed in the KODAK FLEXICOLOR (C-41) process as described in British Journal of Photography Annual, 1988, pp 196-198.

**Table III**

| Multilayer Formulation Variations in AHU and Red Drains | | | | |
|---|---|---|---|---|
| Example | Comp/Inv | Layer E (IL) | Layer F (AHU) | Red Dmin |
| ML-1 | Comp | Present | + BCS (0.15)* | 0.207 |
| ML-2 | Comp | Omit | '' | 0.309 |
| Ml-3 | Comp | Omit | Omit BCS* | 0.197 |
| ML-4 | Comp | Omit | BCS (0.15)* | 0.213 |
| | | | | |
| ML-5 | Inv | Omit | BCS (0.15)* + H-A(0.024) | 0.236 |
| ML-6 | Inv | Omit | BCS (0.15)* + H-A (0.024) | 0.171 |
| ML-7 | Inv | Omit | BCS (0.15)*+ H-A (0.012) | 0.254 |
| ML-8 | Inv | Omit | BCS (0.15)* + H-A (0.024) + ILS-1 (0.162) | 0.212 |

| | | | | |
|---|---|---|---|---|
| *BCS = Black Colloidal Silver | | | | |

Variability of Dmin within a multilayer film is very undesirable. While addition of an interlayer (layer E) between the AHU and imaging layers does decrease red Dmin, it requires an undesirable increase in film thickness as well as an additional layer. As demonstrated by examples ML-2 and ML-3, black colloidal silver (BCS) in the AHU Layer plays a significant role in causing increased red Dmin. Comparison of examples ML-2 and ML-4 shown that red Dmin is further increased when a bleach accelerating releasing coupler (C-3) is present. The addition of the inventive materials like H-A to the AHU layer containing black colloidal silver gave low red Dmin even when the protective interlayer was omitted (Examples ML-6 and ML-4). In addition, materials like H-A were also particularly effective at lowering red Dmin even when a bleach accelerating releasing coupler like C-3 was present in the film element (Examples ML-5 and ML-2). Multilayer Example ML-8 relative to ML-5 shows that compounds like ILS-1 in combination with H-A further improves control of red Dmin.

Multilayer examples ML-9 to ML-13 (with layer E present and with 0.15 black collodial silver in layer F) were prepared, exposed and processed as above to demonstrate the utility of the inventive compounds to reduce increases in Dmin caused by the use of yellow collodial silver (Carey-Lea silver) in the yellow filter layer (YFL). Results are shown in Table IV.

**TABLE IV**

| Multilayer Formulation Variations in YFL and Blue or Green Dmins | | | | |
|---|---|---|---|---|
| Example | Comp/Inv | Layer C (YFL) | Blue Dmin | Green Dmin |
| ML-9 | Comp | YFD-1 | 0.723 | 0.608 |
| ML-10 | Comp | CLS (0.065)* | 0.813 | 0.650 |
| ML-11 | Comp | CLS (0.065)* | 0.872 | 0.651 |
| | | | | |
| ML-12 | Inv | CLS (0.065)* + H-A (0.024) | 0.739 | 0.622 |
| ML-12 | Inv | CLS (0.0.65)* + H-A (0.024) | 0.799 | 0.616 |

| | | | | |
|---|---|---|---|---|
| * CLS = Carey-Lea Silver | | | | |

Comparison of ML-10 to ML-9 demonstrates that CLS in the YFL promotes Dmin increases in neighboring color records relative to dye (YFD-1) where there are no solution physical development effects. The presence of bleach accelerator releasing couplers further increases Dmin (ML-11). Addition of H-A to the YFL containing CLS significantly prevents these Dmin increases.

The element of the invention results not only in lower Dmin and fog in adjacent imaging layers but also causes reduced processing variability in the trade.

The invention has been described in detail with particular reference to preferred embodiments thereof, but it will be understood that variations and modifications can be effected within the scope of the appended claims.

## Claims

1. A color photographic element comprising a non-light sensitive layer containing elemental silver and a nitrogen heterocycle compound having an oil/water partition coefficient ClogP calculated using Medchem 3.54 software of at least 4.5, which compound comprises a ring system of one or more fused rings containing at least one -N-H bond, the ring system comprising a total of at least three nitrogen ring members and the associated bonds; provided that the compound does not contain an -SH group or >C=S group and does not react with an oxidized developer.

2. An element according to claim 1 wherein the nitrogen heterocyle is a benzotriazole.

3. An element according to either of the preceding claims wherein the ClogP of the nitrogen heterocycle is at least 5.5.

4. An element according to any one of the preceding claims wherein the elemental silver is colloidal silver and is neutral in color.

5. An element according to any one of claims 1 to 3 wherein the elemental silver is colloidal silver and is yellow in color.

6. An element according to claim 1 wherein the nitrogen heterocycle is selected from the group consisting of:

7. An element according to any one of the preceding claims wherein the nitrogen heterocycle is selected from the class consisting of:

8. An element according to any one of the preceding claims wherein the layer containing the nitrogen heterocycle compound also contains an interlayer scavenger.

9. An element according to any one of the preceding claims wherein the nitrogen heterocycle compound is dispersed in a hydrophobic organic medium.

10. An element according to any one of the preceding claims which additionally contains at least one bleach accelerator releasing material.

## Patentansprüche

1. Farbfotografisches Element mit einer nicht lichtempfindlichen Schicht, die elementares Silber und eine heterozyklische Stickstoffverbindung mit einem mittels der Medchem 3.54 Software berechneten Öl-/Wasser-Teilungskoeffizienten ClogP von mindestens 4,5 aufweist, wobei die Verbindung ein Ringsystem aus einem oder mehreren kondensierten Ringen umfasst, die mindestens eine -N-H Bindung beinhaltet, und das Ringsystem insgesamt mindestens drei Stickstoff-Ringelemente und die zugehörigen Bindungen umfasst; unter der Voraussetzung, dass die Verbindung keine -SH Gruppe oder >C=S Gruppe enthält und nicht mit einem oxidierten Entwickler reagiert.

2. Farbfotografisches Element nach Anspruch 1, **dadurch gekennzeichnet, dass** die heterozyklische Stickstoffverbindung ein Benzotriazol ist.

3. Farbfotografisches Element nach einem der vorausgehenden Ansprüche, **dadurch gekennzeichnet, dass** der ClogP der heterozyklischen Stickstoffverbindung mindestens 5,5 beträgt.

4. Farbfotografisches Element nach einem der vorausgehenden Ansprüche, **dadurch gekennzeichnet, dass** das elementare Silber ein kolloidales Silber und farbneutral ist.

5. Farbfotografisches Element nach einem der Ansprüche 1 bis 3, **dadurch gekennzeichnet, dass** das elementare Silber ein kolloidales Silber und gelbfarbig ist.

6. Farbfotografisches Element nach Anspruch 1, **dadurch gekennzeichnet, dass** die heterozyklische Stickstoffverbindung aus der Gruppe ausgewählt ist, die folgendes umfasst:

7. Farbfotografisches Element nach einem der vorausgehenden Ansprüche, **dadurch gekennzeichnet, dass** die heterozyklische Stickstoffverbindung aus der Klasse ausgewählt ist, die folgendes umfasst:

8. Farbfotografisches Element nach einem der vorausgehenden Ansprüche, **dadurch gekennzeichnet, dass** die die heterozyklische Stickstoffverbindung enthaltende Schicht zudem ein Zwischenschicht-Maskiermittel umfasst.

9. Farbfotografisches Element nach einem der vorausgehenden Ansprüche, **dadurch gekennzeichnet, dass** die heterozyklische Stickstoffverbindung in einem hydrophoben organischen Medium dispergiert ist.

10. Farbfotografisches Element nach einem der vorausgehenden Ansprüche, das zusätzlich mindestens ein Bleichbeschleuniger-Freisetzungsmaterial enthält.

## Revendications

1. Elément photographique en couleurs comprenant une couche non sensible à la lumière contenant de l'argent élémentaire et un composé hétérocyclique azoté ayant un coefficient de partage huile/eau ClogP calculé en utilisant le logiciel Medchem 3.54 d'au moins 4,5, ledit composé comprenant un système cyclique d'un ou de plusieurs cycles condensés contenant au moins une liaison -N-H, le système cyclique comprenant au total au moins trois chaînons cycliques azotés et les liaisons associées ; à la condition que le composé ne contienne pas de groupe -SH ou >C=S et ne réagisse pas avec un révélateur oxydé.

2. Elément selon la revendication 1, dans lequel l'hétérocycle azoté est un benzotriazole.

3. Elément selon l'une quelconque des revendications précédentes, dans lequel le ClogP de l'hétérocycle azoté est d'au moins 5,5.

4. Elément selon l'une quelconque des revendications précédentes, dans lequel l'argent élémentaire est de l'argent colloïdal et a une couleur neutre.

5. Elément selon l'une quelconque des revendications 1 à 3, dans lequel l'argent élémentaire est de l'argent colloïdal et a une couleur jaune.

6. Elément selon la revendication 1, dans lequel l'hétérocycle azoté est choisi parmi le groupe comprenant :

7. Elément selon l'une quelconque des revendications précédentes, dans lequel l'hétérocycle azoté est choisi parmi le groupe comprenant :

8. Elément selon l'une quelconque des revendications précédentes, dans lequel la couche contenant le composé hétérocyclique azoté contient également un agent d'immobilisation intercouche.

9. Elément selon l'une quelconque des revendications précédentes, dans lequel le composé hétérocyclique azoté est dispersé dans un milieu organique hydrophobe.

10. Elément selon l'une quelconque des revendications précédentes contenant en outre au moins un composé libérant un accélérateur de blanchiment.
